



US005292363A

# United States Patent [19]

Hutcheson

[11] Patent Number: 5,292,363

[45] Date of Patent: Mar. 8, 1994

- [54] PAPERMARKING COMPOSITION, PROCESS USING SAME, AND PAPER PRODUCED THEREFROM
- [75] Inventor: Gary S. Hutcheson, Macon, Ga.
- [73] Assignee: Sequa Chemicals, Inc., Chester, S.C.
- [21] Appl. No.: 16,663
- [22] Filed: Feb. 10, 1993

- 4,826,536 5/1989 Raythatha et al. .... 106/465  
 4,857,126 8/1989 Söremark et al. .... 156/205  
 4,877,539 10/1989 Pioog ..... 252/8.8  
 4,923,566 5/1990 Shawki et al. .... 162/135  
 5,062,922 11/1991 Nakajima et al. .... 162/158  
 5,143,582 9/1992 Arkens et al. .... 162/135

## FOREIGN PATENT DOCUMENTS

- 2314060 3/1973 Fed. Rep. of Germany .... 162/158  
 58-87398 5/1983 Japan ..... 162/158

*Primary Examiner*—David Brunsman  
*Attorney, Agent, or Firm*—Mitchell D. Bittman

## [57] ABSTRACT

A chemical composition for use in the papermaking process to produce a paper having enhanced characteristics of brightness, opaqueness, and sizing is provided. The process using the composition to make the paper and the paper made therefrom are also provided by the present invention. The composition is made by combining an amphoteric softener such as a salt of an amphoteric stearic acid derivative, a cationic softener base, such as the mono- and distearamides of aminoethylethanolamine, an acid, such as acetic acid, a surfactant, such as POE (15) tallow amine, carbamide, and water. In another embodiment, a saccharide may be employed instead of the amphoteric stearic acid derivative, surfactant and carbamide. To speed the production of the composition, a viscosity controlling agent, such as sodium chloride or sodium acetate, may be added thereto. The composition is added to pulp slurry during the papermaking process, and a paper made therefrom exhibits excellent qualities of brightness, opaqueness, water repellency, and dispersibility.

14 Claims, No Drawings

## Related U.S. Application Data

- [63] Continuation of Ser. No. 748,086, Aug. 21, 1991, abandoned.
- [51] Int. Cl.<sup>5</sup> ..... C08L 1/02; C09D 101/02; C09D 7/12
- [52] U.S. Cl. ..... 106/243; 106/203; 106/179; 106/199; 252/8.8; 162/152; 162/158
- [58] Field of Search ..... 106/179, 199, 203, 243; 252/8.8; 162/152, 158

## [56] References Cited

### U.S. PATENT DOCUMENTS

- 2,142,986 1/1939 Arnold, Jr. .... 162/172  
 2,772,967 12/1956 Padbury et al. .... 162/179  
 2,932,602 4/1960 Holgersson et al. .... 162/158  
 3,014,836 12/1961 Proctor, Jr. .... 162/181.8  
 3,096,232 7/1963 Chapman ..... 162/172  
 3,554,862 1/1971 Hervey et al. .... 162/158  
 3,554,863 1/1971 Hervey et al. .... 162/158  
 3,932,210 1/1976 Suzuki et al. .... 162/157.7  
 4,032,473 6/1977 Berg et al. .... 252/358  
 4,075,028 2/1978 Amosov et al. .... 162/186  
 4,225,456 9/1980 Schmidt et al. .... 252/321  
 4,458,080 7/1984 Boehmke et al. .... 162/158  
 4,786,367 11/1988 Bogart et al. .... 162/158  
 4,786,439 11/1988 Pioog et al. .... 252/544  
 4,806,167 2/1989 Raythatha ..... 106/465

**PAPERMARKING COMPOSITION, PROCESS  
USING SAME, AND PAPER PRODUCED  
THEREFROM**

This is a continuation of application Ser. No. 10  
07/748,086, filed Aug. 21, 1991, now abandoned.

**FIELD OF THE INVENTION**

This invention relates to compositions for use in the 10 papermaking process, a papermaking process employing the composition to add opaqueness, brightness, and sizing to the paper, and a paper produced using the composition.

**BACKGROUND OF THE INVENTION**

The quality of paper is often judged by its brightness, opacity, and sizing (or water repellency). Paper producers have long sought to improve these vital characteristics so that an enhanced paper may be obtained.

These three desired characteristics have been obtained in the past by supplying the slurry or furnish with additives prior to the slurry entering the papermaking machine. Various additives are well known in the art. For example, titanium dioxide powder is known to be 25 an excellent whitener. Titanium dioxide, however, is among the most expensive materials that may be added to the slurry. Thus, despite the effectiveness of such material as a brightener, its use is limited and satisfactory replacements have been needed.

Kaolin clay has also been used as a filler in paper to improve brightness in the ultimate product. Generally, the kaolin clay is calcined and then suspended in an aqueous solution prior to being added to the furnish. The clay must be continuously agitated prior to entering the slurry or the solid particles begin to form sediment at the bottoms of the clay holding tanks. Although kaolin clay provides brightness, as well as opacity to the finished paper product, the relative difficulty of adding it to the slurry results in a less than excellent additive. 40

Furthermore, when clay is added to the slurry, the slurry becomes thicker, thus resulting in a slurry having a higher coefficient of friction. The papermaking process using a kaolin-containing slurry therein increases the processing time relative to the time required for 45 processing a pulp slurry not containing kaolin. Moreover, because the kaolin particles are solids and never completely dissolve in the aqueous solutions, the clay tends to clog or foul the mesh of the wire or fabric on the Fourdrinier or other papermaking machine, thereby resulting in a large amount of down time for cleaning the wire or fabric of the machine. Such kaolin-containing products are described in U.S. Pat. No. 3,014,836 to Proctor, Jr. and U.S. Pat. No. 4,826,536 to Raythatha et al.

Hydrated aluminum silicate has also been employed as a clay substitute in the papermaking process. It has properties similar to kaolin clay and, thus, results in the same disadvantages when used to make paper.

Many compositions have been added to the slurry in an attempt to size the paper, i.e., add body to the paper and render the paper water repellent or waterproof. Most known sizes, such as those disclosed in U.S. Pat. No. 2,142,986 to Arnold, Jr. and U.S. Pat. No. 3,096,232 to Chapman, employ a type of wax. For example, Arnold, Jr. discloses that an emulsion of wax in a solution of deacetylated chitin, paraffin waxes, Japan wax, carnauba wax, higher aliphatic alcohols, or synthetic

waxes may be employed as the waterproofing agent in a sizing composition. A softening agent such as aliphatic alcohols containing 12 to 20 carbons is also present in the composition of Arnold, Jr. Chapman discloses the 5 use of paraffin waxes or water-insoluble derivatives of resins for producing aqueous wax emulsions with cationic modified starches.

U.S. Pat. No. 2,772,967 to Padbury shows a paper sized by adding thereto a salt of a high molecular weight composition prepared by reacting a dialkanolamine or trialkanolamine with a long chain fatty acid. The salt is diluted with water to form a dispersion containing a 5% concentration of sizing agent before being applied to the cellulosic fibers. Apparently, such a dilution of strength was necessary heretofore because until the present invention, preparation of the stearamides which would allow the composition to remain pourable at concentrations greater than 5% was unknown. Without the ability to remain in an emulsion and, hence, be

15 poured, concentrations of stearamides approaching those disclosed herein have not been possible for use on pulp fibers. An important feature disclosed by the patent is that the salts are cationic and are, therefore, adsorbed by the anionic cellulosic fibers.

Numerous sizing agents are known. Generally, the known sizes are cationic materials, particularly those used to size fabrics for the textile industry. Although the sizes' cationic nature increases their absorption by the fibers to which they are applied, their cationic nature 30 generally prevents them from being used to the full extent possible in connection with a brightener and opacifying agent. It is well known in the art that although cationic materials often increase sizing, they reduce the brightness of the material to which they are applied. 35 Although this is not generally a problem in the textile industry where sizing is important but opaqueness and brightness may be sacrificed, the use of cationic sizes in the paper industry reduces the quality of the paper made therefrom. Because the addition of cationic sizing agents to paper generally reduces the brightness thereof, cationic sizes have not been heretofore preferred as a size for paper, and in particular, as a size for paper made from recycled pulp which often lacks the inherent brightness of paper made from virgin pulp.

40 Although the prior art shows agents for sizing paper and agents for increasing the brightness and opaqueness of paper, the particular features of the present invention are absent from prior art. The prior art is generally deficient in affording a composition for use in a paper-making process that has the ability to provide sizing to paper without reducing brightness or opacity. Furthermore, the prior art brighteners and opacifying agents fail to allow continuous running of papermaking machines due to the fouling tendencies of the forming fabrics. 45 The present invention, however, overcomes the shortcomings of the prior art in that a composition is disclosed herein for simultaneously increasing the brightness, opacity, and sizing of paper made from a slurry containing the composition.

**SUMMARY OF THE INVENTION**

It is an object of the present invention to provide a composition for adding to paper during the papermaking process so that the resulting paper has enhanced 55 characteristics.

It is another object of the present invention to provide a composition that adds brightness, opacity and sizing to paper to which it is added.

Still another object of the present invention is to provide a composition for adding to the slurry from which paper is formed wherein brightness and opacity of the paper is not sacrificed in favor of sizing.

Another object of the present invention is to provide a composition for brightening, opacifying and sizing a paper which achieves substantially uniform dispersibility on said paper.

Still another object of the present invention is to provide a method for adding a composition to the papermaking process to result in a paper having desirable physical characteristics.

Still another object of the present invention is to provide a process wherein a composition is added to recycled pulp to form a paper having desirable physical characteristics.

Still another object of the present invention is to provide a process for adding a composition to pulp slurry in the papermaking process that will result in a paper having enhanced brightness, opacity, and sizing.

Yet another object of the present invention is to provide a paper having the desirable characteristics of brightness, opacity, and sizing.

Still another object of the present invention is to provide a paper to which a composition has been added during the papermaking process to give the paper enhanced sizing, brightness, and opacity.

Another object of the present invention is to provide a method for preparing an emulsion of fatty acid amides of alkanoldiamines in water where the concentration of fatty acid amides is greater than 5%.

Generally speaking, the present invention is directed to a composition used as an additive to the slurry from which paper is formed, the process of making paper from the additive-containing slurry, and the paper made according to that process. One embodiment of the composition of the present invention employs an amphoteric softener as a brightening agent, a basic cationic softener, an acid, a surfactant, a carbamide, and water. A viscosity control agent may be added to the composition as necessary or desired.

The composition is added to the pulp slurry after the pulp has been bleached to remove lignins and other undesirables and de-inked, if recycled paper pulp is being used, but before the pulp enters into the headbox of a papermaking machine. The composition may be added alone, or in conjunction with other brighteners, opacifying agents, and sizes. For example, in one embodiment of the invention, the composition hereof may be added in conjunction with papermaking clays such as kaolin.

The composition may be added to any pulp slurry to obtain the desired physical characteristics and is especially useful for enhancing the characteristics of paper made from recycled pulp. The amount of composition, as well as the amounts of each component in the composition, will vary depending on the characteristics and types of pulp slurry to which the composition is added. As is well known, different sources of pulp have different peculiarities that attribute to their ability to be brightened, made more opaque and more water resistant, and easily processed. For instance, some pulp requires a higher concentration of brightening and opacifying agents than others to produce a finished paper product having identical characteristics.

In one embodiment of the invention disclosed herein, the amphoteric softener, which contributes to the brightening of the paper, is a fatty acid amphoglycinate,

such as sodium stearoamphoglycinate. Generally, the amphoteric softener is in salt form to increase its solubility.

The cationic softener base in this embodiment includes mono- and distearamides of aminoethylethanolamine and mixtures thereof. This component contributes to the opacity and sizing, as well as the brightness, of the paper made according to the present invention. Preferably, the stearamides are dissolved by a weak organic acid such as acetic acid so that an acidic reaction environment is maintained wherein the pH is preferably between about 4 and about 5.

In making the present embodiment of the composition, the amphoteric softener and cationic softener base are charged to a mixing tank along with a surfactant and water. The components are heated to between about 196° C. and 204° C. and agitated until all the solid components are melted and substantially dispersed. Thereupon, the acid is added and agitation continued. A viscosity controlling agent may be added to reduce the viscosity of the mixture. The composition is then cooled with water. After sufficient cooling, urea is added and agitation continued until all the urea is dissolved. The composition is then added to pulp slurry and paper having the desired characteristics of brightness, opacity, and water repellency is produced therefrom.

In another embodiment of the present composition, the reaction product of a saccharide, such as a sucrose derivative, and an acid may replace the amphoteric softener, surfactant, and urea. In this embodiment, sucrose is reacted with an acid to form a product that provides added brightness and sizing to the paper made utilizing the composition. This reaction product also acts as the surfactant in this embodiment by lowering the surface tension of the composition and allowing the components thereof to remain in an emulsion.

The paper obtained from the papermaking process employing a slurry containing the present inventive composition exhibits excellent brightness, opacity, and sizing characteristics. Unlike prior art additives that employ cationic components, brightness and opacity of paper made with the claimed composition are not sacrificed in favor of sizing.

#### DESCRIPTION OF PREFERRED EMBODIMENTS

A composition for use in the papermaking process such that opaqueness, brightness, and sizing is added to the paper, a papermaking process employing same, and a paper produced from same are provided. Generically, this composition comprises an amphoteric softener, a cationic softener base, an acid for controlling pH, a surfactant, carbamide, and water. In another embodiment of the composition, the amphoteric softener, urea, and surfactant may be eliminated and replaced by a saccharide brightening and sizing agent. Additionally, a viscosity controlling agent may be employed as necessary or desired to aid in production of any of the particular embodiments of the composition.

The composition is added to a pulp slurry after the pulp has been bleached but before the pulp enters into the headbox of a papermaking machine. The composition may be added alone, or in conjunction with other brighteners, opacifying agents, sizes and additives employed in the papermaking process.

The type of pulp slurry to which the composition may be added is unimportant. In fact, the make-up of the composition may be varied depending on the type of

cellulosic fibers from which the pulp slurry is made. For instance, if the pulp is inherently dark and requires more brightening, the amount of amphoteric softener or saccharide in the composition may be increased to add brightness to the paper. On the other hand, if the paper produced from the pulp lacks a sufficient degree of water repellency, the amount of cationic softener base or the saccharide may be increased to improve sizing. To increase opaqueness, additional amounts of the cationic softener base and/or the carbamide may be employed. In addition, the use of pulp which has been recycled from papers may require other adjustments to the composition, particularly when the recycled pulp is dark or otherwise discolored. All such adjustments to the composition may be easily made by one of ordinary skill in the art according to the invention disclosed herein.

The pulp to which the composition is added is made into a slurry using conventional techniques. After formation, the slurry is stored in holding tanks or fed to a papermaking machine, such as a Fourdrinier machine, in a conventional manner. The pulp may be bleached to remove unwanted pollutants such as lignin and de-inked if pulp made from recycled paper is used. The papermaking composition disclosed herein may be added either to the slurry when it is in the holding tank or may be added to the slurry as it moves along to the headbox of the papermaking machine. Preferably, the composition is sprayed onto the flowing pulp as it travels to the headbox.

When the slurry containing the composition reaches the headbox of the papermaking machine, paper is formed therefrom using conventional papermaking techniques and materials. The paper produced according to the present invention exhibits excellent characteristics of opaqueness, brightness, and opacity.

Moreover, the addition of the composition to the pulp slurry does not cause substantial negative effects on the slurry's movement through the papermaking process and, in fact, actually decreases the coefficient of friction for the slurries to which it is added. Slurries having high coefficients of friction result in increased drag in the meshes and pulp flow, thus hindering the speed of the papermaking process. Slurries to which clays have been added usually have high coefficients of friction and, as a result, can only run at lower speeds.

In a further embodiment of the present invention, other materials may be added in conjunction with the composition. For instance, kaolin clay may be added in addition to the inventive composition so that the paper made therefrom exhibits increased opaqueness. Other additives which are well known in the art may also be added in conjunction with the composition disclosed herein.

5  
The amphoteric softener used in making the claimed composition is preferably in a salt form to enhance solubility thereof. The amphoteric softeners contribute to the brightening of the paper made with the composition. The amphoteric capability of this component allows for different ionic structures in different environments. As described herein, the amphoteric softener maintains a cationic nature in the acidic environment of the present composition which contributes to the reaction activity of the cationic softener base described below. The amphoteric softener used in the composition preferably is a fatty acid derivative having from 12 to 18 carbons. The salts of stearic acid amphoglycinate derivatives, and particularly sodium stearoamphoglyci- 6

inate, most advantageously exhibit the preferred qualities of the amphoteric softener component and are also readily available in the marketplace.

5 The cationic softener base contributes primarily to the paper's opacity and sizing. Although the preferred cationic softener bases include the mono- and distear-  
10 amides of aminoethanolamines and mixtures thereof, any of the fatty acid amides may be used and the cationic softener is not limited to the stearic acid amides. Amino-  
15 ethanolamines available include aminoethylethanolamine, aminobutylethanolamine, aminomethylethanolamine, aminopropylethanolamine and the other alkyl-  
substituted aminoethanolamines. The preferred steara-  
20 mide derivatives are aminoethylethanolamine monostearyl amide and aminoethylethanolamine distearyl amide which are mono- and di-substituted fatty acid amides of alkanoldiamines. Other cationic softener bases such as derivatives of imidazole, and in particular imidazoline, may also be used in the present composi-  
25 tion.

The preferred cationic softener bases have the general formula



30 wherein  $R_1$  represents a  $CH_{2n+1}$



35 group wherein n is a number from 11 to 17, wherein R<sub>2</sub> represents either a



group wherein  $n$  is a number from 11 to 17 or hydrogen, wherein  $R_3$  represents an alkyl group, and wherein  $R_4$  represents an aliphatic alcohol. Compounds according to this general formula are the reaction products formed from fatty acids and diamines, and, more specifically, are the reaction products of fatty acids and alkanoldiamines (diamine aliphatic alcohols). The chosen fatty acid and chosen alkanoldiamine are mixed and heated at temperatures of 160°-200° C. to produce the monos-tearamides, distearamides, and mixtures thereof. The most preferred cationic softener bases have the formulas



၁၀၁



which represent the mono- and distearamides of amino-ethylethanolamine.

Preferably, the cationic softener base used in the present composition will predominantly consist of di-substituted fatty acid amides, particularly distearamides. 5 Because the di-substituted amides have two fatty acid amide groups as opposed to the mono-substituted amides which have only one fatty acid amide group, the di-substituted amides are more active cationic bases.

Particularly, the distearamides show a stronger affinity for the cellulosic fibers to which they are adsorbed.

In addition, it is preferred that the particle size of the cationic softener base be as small as possible. The cationic softener base made according to Example 1 herein is a hard solid substance. In order for the cationic softener to remain in an emulsified state as in the composition described herein, intense agitation and heating is required. Moreover, it is highly desirable that the papers produced according to the present invention have substantially uniform brightness, opaqueness, and sizing over its entire surface. Smaller particle sizes aid in the dispersibility of the particles within the slurry so that the desired characteristics are uniform throughout the paper. These smaller particle sizes may be obtained by either homogenizing the product in a high speed mixer or by rapidly cooling the composition from the high temperature at which the cationic softener base is formed as described herein.

A weak acid is preferred to dissolve the solid cationic softener base. The acid maintains an acidic pH preferably within the range of from about 4 to about 5 during the making of the composition. The acid acts as a catalyst by creating an acidic environment wherein the cationic softener base exhibits increased reactivity and the amphoteric softener, when employed, maintains a cationic nature. Weak organic acids such as acetic acid or formic acid are especially preferred in the composition. Strong acids, of course, may be used to control the pH, but cost and safety considerations may restrict their use.

A preferred surfactant used in the present invention is an ethoxylated surfactant such as POE (15) tallow amine. The surfactant further contributes to the desired dispersibility of the components. If the amount of surfactant added is excessive, the sizing capability of the composition will be adversely affected. In the absence of a surfactant, the paper may be of a poor quality due to the decreased dispersibility of the composition, which results in spots or specks on the paper indicating a lack of uniform dispersion as discussed above.

The carbamide, preferably urea, contributes to opacity of the paper. Other carbamide derivatives may be used in the invention as long as they dissolve as the composition is being made and do not detract from the opacity of the finished paper.

In another embodiment, the composition employs a saccharide derivative as a brightener and size. This embodiment contains the previously described cationic softener base but, because the saccharide derivative acts as a surfactant to allow adequate dispersion, the POE (15) tallow amine may be eliminated. In addition, the carbamide may also be eliminated in this embodiment because the paper to which this embodiment is added may exhibit the desired opacity. When employed, the saccharide component nearly doubles the effective sizing capability of the composition.

Preferably, a viscosity controlling agent such as a salt is added during the production of the papermaking composition. Generally, the sodium salts and chloride salts are known viscosity controlling agents. Preferred salts include sodium acetate and sodium chloride. This component may be deleted, but the processing time for creating the composition will be substantially increased.

The present invention may be better understood by reference to the following examples.

### EXAMPLE 1

Mono- and distearamides of aminoethylethanolamine are made by reacting stearic acid with aminoethylethanol amine. 1845 grams of stearic acid (65% stearic acid and 35% palmitic acid) and 405 grams of aminoethylethanol amine are charged to a reactor and sparged with nitrogen at a rate of 10 ft<sup>3</sup>/min. Using slow agitation, the temperature of the reactor is raised to between about 385° F. and about 400° F. (196°-204° C.) and preferably about 392° F. (200° C.), and held at such a temperature for about 45 minutes. The product is then allowed to cool at room temperature. The liquid weight percentages of the components used in making the stearamides are 82.83% stearic acid and 17.17% aminoethylethanol amine.

### EXAMPLE 2

A composition of the present invention is prepared as follows. 1075 grams of sodium stearoamphoglycinate, 3400 grams of the mono- and distearamides of aminoethylethanol amine made according to Example 1, 325 grams of POE (15) tallow amine (TAM 15 obtained from Henkel Co.) and 9996 grams of water are charged to a mixing tank equipped with an agitator. Heating and agitation are begun, and the mixture is heated to between 195°-205° F. (91°-96° C.) and held at this temperature for approximately one hour. When all the solid components in the mixing tank are melted and homogeneously dispersed, 499 grams of acetic acid is added and agitation continued for about 15 to 30 minutes. After such agitation, about 100 grams of sodium chloride is added and agitation continued for another 30 minutes. Thereafter, heating is discontinued, cooling water is cycled through the jacket coils surrounding the mixing tank, and 8330 grams of additional water is added to the mixing tank to cool the contents. The temperature of the dispersion is monitored until it reaches 140° F. (60° C.). 6000 grams of urea is then added to the mixing tank with cooling and agitation continuing until the temperature of the constituents reaches about 110°-115° F. (42°-46° C.) and all the carbamide dissolved.

The dry weight percentages of the components are shown below:

| Component                                                                                          | Dry Weight Percent of Component |
|----------------------------------------------------------------------------------------------------|---------------------------------|
| Amphoteric Softener<br>(sodium stearoamphoglycinate)                                               | 3.60%                           |
| Cationic Softener<br>Base<br>(mono- and distearamides of aminoethylethanolamine made in Example 1) | 11.50%                          |
| Viscosity Controlling<br>Agent<br>(sodium chloride)                                                | 0.34%                           |
| Acid<br>(acetic acid)                                                                              | 1.70%                           |
| Surfactant<br>(POE (15) tallow amine)                                                              | 1.10%                           |
| Carbamide                                                                                          | 20.30%                          |
| Water                                                                                              | 61.50%                          |

### EXAMPLE 3

The process and components described in Example 2 were employed in making a further embodiment of the inventive composition. In this composition, dry weight percentages used were as follows: amphoteric softener

(sodium stearoamphoglycinate) about 1.13%, cationic softener base (mono- and distearamides of aminoethylethanolamine) about 8.00%, viscosity controlling agent (sodium chloride) about .25%, acid (acetic acid) about 0.98%, surfactant (POE (15) tallow amine) about 0.75%, carbamide (urea) about 14.00%, and water comprising the remaining about 74.89% by weight.

It has also been found through further refining of the composition that the amphoteric softener, preferably sodium stearoamphoglycinate, should be in a range of between about 0.5% to about 4%. The cationic softener base, preferably the mono- and distearamides of aminoethylethanolamine made according to Example 1, should be present in an amount of about 7.5% to about 13%. The viscosity controlling agent should be present in an amount of about 0.25 to about 0.35%. The acid, preferably acetic or formic acid, should be present in an amount at least of about 0.9% so that the pH of the mixture is controlled between about 4 and about 5. The non-ionic surfactant, preferably POE (15) tallow amine, should be present in an amount of at least about 0.75%. The carbamide used in the composition should be within the range of from about 10% to about 25% and the water should be in a range of from about 60% to about 75%.

#### EXAMPLE 4

A composition made according to Example 2 was added to a pulp slurry as the pulp slurry was transported along a feeding mechanism to the headbox of a 30 Fourdrinier machine. The composition was added at a rate of 3 to 3½ gallons per minute, and paper produced therefrom exhibited the desired characteristics. The coefficient of friction of the slurry after adding the composition was measured and determined to be 0.3. 35

#### EXAMPLE 5

A composition made according to the process described above in Example 2 was added to a pulp slurry as the pulp slurry was transported along a feeding mechanism to the headbox of a Fourdrinier machine. The composition was added at a rate of 2.8 gallons per minute, and paper produced therefrom exhibited the preferred characteristics. 40

#### EXAMPLE 6

The composition made according to Example 2 was added to a pulp slurry as it was transported to the headbox at a rate of 5 gallons per minute. The paper produced according to this example showed increased opacity and sizing but a similar brightness compared to the paper produced according to Example 4. 50

#### EXAMPLE 7

A composition made according to the process of Example 2 was added to a pulp slurry at a rate of 2 gallons per minute. In addition, a 33% aqueous solution of kaolin clay was added coincidentally with the paper-making additive to the slurry at a rate of 8 gallons per minute and paper was produced therefrom. Although the paper exhibited the desired characteristics, the coefficient of friction of the slurry after adding the composition and the clay was determined to be 0.7. 60

A 33% aqueous slurry of kaolin clay alone was added to a pulp slurry as it traveled to a Fourdrinier machine so that paper produced therefrom could be compared to paper made with the present invention. To produce paper having brightness characteristics comparable to

those exhibited by the paper made according to Example 4, kaolin clay was added to the slurry at a rate of about 12 gallons per minute.

When adding the composition to a pulp slurry as described in Example 4, without the addition of kaolin clay, the Fourdrinier machine exhibited excellent runability, less drag, less power requirements, and overall smoother operation than the machine did when kaolin clay was added to the slurry. These characteristics add to the overall operational printability of the paper made using the present composition.

The coefficient of friction for the pulp slurry without the addition of any kaolin clay or the addition of the inventive composition was also measured. The coefficient for the slurry without any such additives was 0.5. As evidenced by the low coefficient of friction noted in Example 4, addition of the inventive composition to a pulp slurry actually decreases the amount of drag as compared to a papermaking process using a pulp slurry in which no additives are employed.

#### EXAMPLE 8

Sucroseoxyacetate for use as a component in compositions according to the present invention was made as follows. 600 grams of 84% acetic acid was added to 400 grams of sucrose in a vessel equipped with an agitator as in the preceding examples. The mixture was agitated and heated to about 135°-140° F. (57°-60° C.). Temperature was then held until titrations indicated one gram of reaction mixture dissolved in 100 mls. of water (6.0 to 7.0 mls. of 1.0 M sodium hydroxide to titrate to phenolphthalein endpoint). The resulting sucroseoxyacetate was then allowed to cool for further use.

#### EXAMPLE 9

An embodiment of the present invention employing a saccharide as a brightener and size is made as follows. 110 grams of the mono- and distearamides and mixtures thereof made according to Example 1 are heated to about 212° F. (100° C.) until a melt thereof is formed. An emulsion is created by adding water to the melt followed by agitation. Two grams of sodium acetate is added to the mixing tank after the emulsion thins and cools to about 180°-190° F. (82°-88° C.). Cooling and agitation are continued until the temperature of the emulsion drops to below about 165° F. (74° C.), whereupon 50 grams of sucroseoxyacetate made according to Example 8 is added to the mixing tank. Agitation continues for about 30 minutes and additional water is metered into the mixing tank so that the total amount of the water added totals about 838 grams.

Weight percentages of the components used in the present example are set forth below:

| Component                                                                                    | Dry Weight Percent of Component |
|----------------------------------------------------------------------------------------------|---------------------------------|
| Cationic Softener Base (mono- and distearamides of aminoethylethanolamine made in Example 1) | 11.00%                          |
| Sucroseoxyacetate (made in Example 8)                                                        | 5.00%                           |
| Viscosity Controlling Agent (sodium acetate)                                                 | 0.20%                           |
| Water                                                                                        | 83.80%                          |

## EXAMPLE 10

A composition of Example 9 was added to a pulp slurry prior to entering a papermaking machine headbox at a rate of 3-3.5 gallons per minute and a paper having the desired characteristics was formed therefrom.

## EXAMPLE 11

A composition made according to the process of Example 9 was added to a pulp slurry at a rate of about 2½ gallons per minute in addition to a 33% aqueous solution of kaolin clay which was added at a rate of 8 gallons per minute. The paper produced therefrom exhibited the desired characteristics but the slurry had a coefficient of friction of 0.7.

As explained above, the making of stearamides according to Example 1 produces a hard solid compound. If the preferred dispersibility of the composition is to be obtained, the cationic softener base requires homogenization prior to combining with the other components of the composition. One method of homogenization employs vigorous agitation and heating. Instead of allowing the mono- and distearamides of aminoethylethanolamine to cool to room temperature as described in Example 1, the stearamides are only allowed to cool to about 200° F. (93° C.). The cationic softener is held at this temperature, which is just below the boiling point of the liquid, until it is combined with the other components. The other components of the composition are preheated to about 190° F. (88° C.) and the required amount of cationic softener base is added thereto to comprise the appropriate percentage within the composition. The composition is then held at about 200° F. and vigorously agitated for about one hour. This results in an emulsion having substantially uniform small particle size so that good dispersion of the composition with respect to the pulp slurry is achieved thereby.

Alternatively, the composition may be homogenized to provide the good dispersion characteristics by rapid super cooling of the composition. Using this method, the stearamides are held at a temperature of about 200° F. and then transferred in the appropriate amount to the preheated remaining component mixture. After achieving a temperature of about 200° F., the mixture is rapidly cooled to room temperature by subjecting the mixture to dry ice or other super cooling methods. This results in an emulsion having substantially uniform small particle size throughout. Such super cooling methods may include the use of storage tanks being cooled by circulating freon, but the method of making the present composition is not limited to a particular method of super cooling.

The super cooling of the composition may be employed in addition to the homogenization by agitation described above, or may be used in lieu of such agitation. Examples of creating the preferred homogenous composition follow.

## EXAMPLE 12

Mono- and distearamides of aminoethylethanolamine are made generally according to Example 1 above, but instead of allowing the product to cool to room temperature, the stearamides are only allowed to cool to about 200° F. (93° C.). The components of the composition in the amounts and percentages described in Example 2 are preheated to about 190° F. (88° C.) in a Shear Hill Mixer manufactured by Hill Manufacturing Company.

An amount of the mono- and distearamides of aminoethylethanolamine sufficient to comprise about 11.5% dry weight of the final composition (3400 grams) is added to the mixer. High-speed agitation is begun and continued at 200° F. for about one hour. The resulting composition achieves the preferred dispersibility with respect to the slurry when added thereto as described in Examples 4-7.

In the other embodiment described in Example 9 herein, the sucroseoxyacetate, viscosity controlling agent, and water are preheated in the Shear Hill Mixer. The cationic softener base in the stated amount is, likewise, maintained at a temperature of about 200° F. after creation thereof and is added to these other components in the mixer. Agitation continues at about 200° F. for about one hour to achieve a preferred composition having the desirable characteristics of brightness, opacity, water repellency, and uniform dispersibility throughout the slurry.

## EXAMPLE 13

A preferred composition of the present invention may alternatively be made by employing super-cooling to achieve the desired dispersibility of the composition with respect to the slurry. The mono- and distearamides of aminoethylethanolamine are made generally according to the process of Example 1. Instead of allowing the mixture to cool to room temperature, however, the emulsion is allowed to cool only to about 200° F. (93° C.). The remaining components of the composition in the amounts described in Example 2 are preheated to about 190° F. The stearamides and other components are then mixed and agitated at about 200° F. for about 10 minutes. After such mixing, the mixing vessel is rapidly cooled using a dry ice pack so that the temperature of the emulsion is reduced to room temperature or below in about 10 minutes or less. This cooling process also results in a composition having the desired dispersion characteristics.

As mentioned above, the rapid super-cooling of the mixture may be employed in addition to the one-hour agitation in the mixer as described in Example 12 or may, alternatively, be employed in lieu of such agitation. Preferably, however, the prolonged high-speed agitation of Example 12 will be combined with the rapid super cooling described in Example 13 to achieve the preferred product. It will also be appreciated by those of ordinary skill in the art that other methods and apparatus may be employed to achieve such super cooling. It will also be understood by those of ordinary skill in the art that the super agitation and/or super cooling described in Examples 12 and 13 may be used in producing any of the various embodiments of the present invention to achieve good dispersibility of the composition with respect to the paper made from the slurry.

By employing the processes described in Examples 12 and 13, a method of preparing an emulsion of fatty acid amides of an alkanoldiamine in water where the concentration of fatty acid amides is greater than 5% is provided. As explained earlier, prior art methods of preparing emulsions of fatty acid amides employed in the present composition in water have been limited to concentrations of 5% or less. By providing the fatty acid amides of the alkanoldiamine at a temperature of about 200° F., mixing the fatty acid amides with the liquid serving as an emulsifier until the fatty acid amides are dispersed therein and then rapidly cooling the mixture of fatty acid amides and emulsifier such that the fatty

acid amides remain in an emulsified state with respect to the emulsifier results in the ability to provide an emulsion where the fatty acid amides' concentration is greater than 5%. Of course, such rapid cooling processes described in Example 13 may be combined with the super agitation process of Example 12 to provide for even greater percentages of fatty acid amides and emulsion.

The opacity, brightness and water repellency of the paper produced according to Examples 4 and 10 were measured and compared to paper made from a slurry from pulp of a similar source to which no brightening, opaquing, or sizing agents had been added. The results are shown below:

|                     | Opacity*  | Brightness* | Size**  |
|---------------------|-----------|-------------|---------|
| Plain Paper         | 90.5-91.0 | 58-59       | instant |
| Paper of Example 4  | 94.0-94.5 | 58-59       | 50 sec. |
| Paper of Example 10 | 94.0-94.5 | 60-61       | 90 sec. |

\*Opacity and brightness were measured using a Technidyne Technibrite Micro TB-1C. Measurements are given in TAPPI standard units.

\*\*Sizing was measured using the standard water drop test.

One with skill in the art will appreciate the fact that the rate of adding any of the embodiments of the inventive composition to a pulp slurry will vary depending on the peculiarities of the pulp, the characteristics desired in the paper made therefrom, and the capabilities of the papermaking machine and slurry feeding mechanism. As previously explained, these factors will also influence the exact amounts of each component used in producing the papermaking composition. Testing, however, showed that the preferred rate of adding the composition to achieve optimal characteristics and a low coefficient of friction was between 2 and 5 gallons per minute.

Although preferred embodiments of the invention have been described using specific terms, devices, concentrations, and methods, such description is for illustrative purposes only, and it is to be understood that changes and variations may be made without departing from the spirit or the scope of the following claims.

What is claimed is:

1. A composition for addition to a pulp slurry of cellulose fibers in a papermaking process for enhancing brightness, opacity and sizing of a paper produced from said pulp comprising an amphoteric softener, a cationic softener, an acid, a surfactant and a carbamide.

2. A composition for addition to a pulp slurry of cellulose fibers for the formation of paper for enhancing brightness, opacity and sizing of a paper produced from said pulp comprising an amphoteric softener selected from the group consisting of salts of amphoteric fatty acid derivatives, a cationic softener base selected from the group consisting of reaction products formed from fatty acids and diamines, an acid, a surfactant, and a carbamide.

3. The composition as defined in claim 2 wherein said amphoteric softener is sodium stearoamphoglycinate, said cationic softener base is selected from the group consisting of aminoethylethanolamine monostearylamide, aminoethylethanolamine distearylamine, mixtures of aminoethylethanolamine monostearylamide and aminoethylethanolamine distearylamine, and imidazoline, said acid is selected from the group consisting of

acetic acid and formic acid, said surfactant is ethoxylated surfactant, and said carbamide is urea.

4. The composition as defined in claim 3 further comprising an agent for controlling viscosity.

5. The composition as defined in claim 2 wherein said amphoteric softener is present in an amount from about 0.5% to about 4% by weight, said cationic softener base is present in an amount from about 7.5% to about 13% by weight, said acid is present in an amount of at least about 0.9% by weight so that the pH of the composition is between about 4 and about 5, said surfactant is present in an amount of at least about 0.75% by weight, and said carbamide is present in an amount from about 10% to about 25% by weight.

6. A composition for addition to a pulp slurry of cellulose fibers for the formation of paper for enhancing brightness, opacity and sizing of a paper produced from said pulp comprising a cationic softener base selected from the group consisting of reaction products formed from the reaction of fatty acids and alkanoldiamines and a brightening and sizing agent selected from the group consisting of reaction products formed from the reaction of a saccharide and an acid.

7. The composition as defined in claim 6 wherein said cationic softener base is selected from the group consisting of aminoethylethanolamine monostearylamide, aminoethylethanolamine distearylamine, mixtures of aminoethylethanolamine monostearylamide and aminoethylethanolamine distearylamine, and imidazoline, and said brightening and sizing agent is sucroseoxacetate.

8. The composition as defined in claim 6 further comprising a viscosity controlling agent.

9. The composition as defined in claim 8 wherein said viscosity controlling agent is selected from the group consisting of sodium chloride and sodium acetate.

10. The composition as defined in claim 6 comprising from about 9.0% to about 13.00% by weight cationic softener and about 3.5% to about 6.5% by weight brightening and sizing agent.

11. A method of preparing an emulsion of fatty acid amides of an alkanoldiamine in water where the concentration of fatty acid amides is greater than 5% comprising the steps of:

45 providing said fatty acid amides of an alkanoldiamine at a temperature of about 200° F.; mixing said fatty acid amides with the liquid serving as an emulsifier until said fatty acid amides are dispersed therein; rapidly cooling said mixture of fatty acid amides and emulsifier such that said fatty acid amides will remain in an emulsified state with respect to said emulsifier.

12. The method as defined in claim 11 wherein said fatty acid amides are selected from the group consisting of aminoethylethanolamine monostearylamide, aminoethylethanolamine distearylamine, mixtures of aminoethylethanolamine monostearylamide and aminoethylethanolamine distearylamine, and imidazoline.

13. The method as defined in claim 11 wherein said rapid cooling is carried out by applying a dry ice pack to said mixture.

14. The method as defined in claim 11 further comprising the step of vigorously agitating said mixture for about one hour.

\* \* \* \* \*